

Jan. 17, 1933.

T. K. COX

1,894,671

## METHOD OF COATING ARTICLES

Filed June 8, 1929

Fig. 1.



Fig. 2.



Fig. 3.



Inventor  
Thomas K. COX  
By H. Patterson: Atty.

## UNITED STATES PATENT OFFICE

THOMAS KING COX, OF CHICAGO, ILLINOIS, ASSIGNOR TO WESTERN ELECTRIC COMPANY, INCORPORATED, OF NEW YORK, N. Y., A CORPORATION OF NEW YORK

## METHOD OF COATING ARTICLES

Application filed June 8, 1929. Serial No. 369,351.

This invention relates to a method of coating articles, and more particularly to a method of treating wire to promote adherence thereto of an insulating coating.

5 An object of the invention is to provide a simple and efficient method of treating articles to promote the adherence thereto of a coating material.

According to the general features of the 10 invention, the article to be coated is subjected to a bath of an organic acid, and a coating of insulating compound is subsequently applied to the article. Due to the action of the acid a firm bond is formed therebetween 15 which is substantially integral with both the coating and the article.

The invention will be readily understood 20 from the following specification when read in conjunction with the accompanying drawing, in which

Fig. 1 is a fragmentary plan view of an apparatus which may be employed in practicing the invention;

Fig. 2 is a fragmentary elevation thereof, 25 and

Fig. 3 is an enlarged cross sectional view of an insulated copper wire formed in accordance with the invention.

The apparatus shown consists of an extruding head 10 which is secured by bolts 11 to an insulation extruding machine 12 (shown broken away) of any well known type, wherein the materials comprising the insulation are macerated, heated, and mixed 30 into a warm, homogeneous mass. A nozzle 14 projects outwardly from the extruding head 10 and is adapted to receive at one end a tinned copper wire 15 travelling in a horizontal path and, as the wire passes from the 35 other end of the nozzle, to extrude upon it a cylindrical coating 16 of insulating compound. Although tinned copper wire is preferably used, the invention is also applicable to all substances which react with an 40 organic acid to form salts soluble in coating materials such as hydrocarbons and gum exudations. Mounted upon the extruding head 10 by bolts 17 in such manner as to be located beneath the wire 15 before its passage 45 into the nozzle 14 is a container 18, composed

of any suitable acid-resisting material. The container 18 comprises a basin 19 and an integral projecting drain 20 having a bottom inclined to direct into the basin portion liquid deposited thereon. The basin portion contains a supply of oleic acid 23 which saturates a sponge 24 resting therein, the latter being of sufficient size to protrude above the sides of the container 18 and be maintained at all times in contact with the moving wire 55 15. The nozzle 14 is fitted at the receiving end thereof with a gland 26 which is of such construction as will permit it to bear upon the periphery of the wire 15 and remove therefrom the excess of acid, which drips into 60 the drain 20 and is thereby returned to the supply 23.

The insulating compound extruded upon the wire may be composed; for example, of 65 25% reclaimed rubber, 20% smoked sheet rubber, 5% mineral rubber, 5% zinc oxide, 2% sulphur, 2% pine tar, and 41% whiting. The proportions and materials used in the compound may be widely varied, in accordance with established practice depending upon 70 the character of insulation desired. It is essential, however, that the compound include a substantial proportion of a substance which will dissolve metallic salts such as tin oleate. Examples of such materials, in addition to the 75 compound described above, are gutta percha, paraffins, and other hydrocarbons, and certain gum exudates useful as insulators, such as balata.

After treatment in accordance with the 80 step described above, it has been observed that the wire upon receiving a deposition of insulating material will, upon subsequent vulcanization thereon of the insulating material, 85 be found to be securely bonded to such insulation. Although it is difficult to observe exactly the progress of the reactions producing this bond, it is probably due to the fact that the action of the acid upon the metal surface of the wire forms a film of salts of 90 tin, or tin oleate. These salts, being soluble in the warm compound, create a film 27 between the metal and the compound which is 95 essentially integral with both. Upon cooling after vulcanization the bond will be 100

found to resist strongly strains such as would normally strip insulation applied in the old method therefrom.

In addition to oleic acid, advantageous results may be secured by the use, in lieu thereof, of other organic acids having a high molecular weight such as palmitic and stearic acids. It is also possible to employ organic acids having lower molecular weights, such as 10 acetic acid and formic acid. In the latter cases, however, it is desirable to allow a longer time for completion of the reaction described.

The foregoing describes but one embodiment of the method of securing a firm adherence of a coating to an article. The invention is capable of many other embodiments not mentioned above, and it is therefore desired that the scope of the invention be 20 not limited except by the scope of the appended claims.

What is claimed is:

1. The method of securing the adhesion of a rubber compound to a metallic body which 25 consists in depositing thereon a film of an acid of the organic class consisting of formic, acetic, oleic and palmitic acids, applying thereon the compound while in a plastic state, and thereafter vulcanizing the compound to 30 the metallic body.

2. The method of insulating an electrical conductor which consists in depositing thereon oleic acid to form a film, subsequently depositing upon the film a hydrocarbon compound 35 containing sulphur, and thereafter vulcanizing the compound to the conductor.

3. The method of insulating an electrical conductor which consists in wetting the conductor with oleic acid, depositing upon the 40 acid covered conductor a rubber compound while in a plastic state, and thereafter vulcanizing the compound to the conductor.

4. The method of securing the adhesion of a rubber compound to a tinned metallic body 45 which consists in depositing thereon a quantity of oleic acid, applying the compound to said metallic body while in a plastic state, and thereafter vulcanizing the compound to said metallic body.

50 In witness whereof, I hereunto subscribe my name this 28th day of May A. D., 1929.

THOMAS KING COX.